



US005198131A

**United States Patent** [19]  
**Hsu et al.**

[11] **Patent Number:** **5,198,131**  
[45] **Date of Patent:** **Mar. 30, 1993**

[54] **DIALKANO- AND TRIALKANOL  
AMINE-DERIVED THIOESTER  
MULTIFUNCTIONAL ANTIWEAR  
ADDITIVES**

[75] Inventors: **Shih-Ying Hsu, Morrisville, Pa.;  
Andrew G. Horodysky, Cherry Hill,  
N.J.**

[73] Assignee: **Mobil Oil Corporation, Fairfax, Va.**

[21] Appl. No.: **815,018**

[22] Filed: **Dec. 27, 1991**

[51] Int. Cl.<sup>5</sup> ..... **C10M 135/26; C07C 323/52**

[52] U.S. Cl. ..... **252/47.5; 560/147**

[58] Field of Search ..... **252/47.5; 560/147**

[56] **References Cited**

**U.S. PATENT DOCUMENTS**

2,223,130 11/1940 Prutton ..... 252/47.5  
2,238,478 4/1941 Elsmere ..... 252/47.5

2,257,752 10/1941 Lincoln et al. ..... 252/47.5  
2,268,185 12/1941 Burke et al. ..... 560/147  
2,330,239 9/1943 Prutton ..... 252/47.5  
2,614,980 10/1952 Lytle ..... 252/47.5  
4,201,684 5/1980 Malec ..... 252/47.5  
4,515,687 5/1985 Bresson et al. ..... 252/61  
4,761,482 8/1988 Karol ..... 548/142  
4,863,534 9/1989 Forsberg ..... 149/2  
4,919,831 3/1990 Horodysky ..... 252/47.5  
4,994,150 2/1991 Shaw ..... 560/147

*Primary Examiner*—Prince Willis, Jr.

*Assistant Examiner*—Alan D. Diamond

*Attorney, Agent, or Firm*—Alexander J. McKillop;  
Malcolm D. Keen; Howard M. Flournoy

[57] **ABSTRACT**

Dialkanol- and trialkanol amine-derived thioesters have been found to be effective multifunctional antiwear additives for lubricants and fuels.

**16 Claims, No Drawings**

**DIALKANO- AND TRIALKANOL  
AMINE-DERIVED THIOESTER  
MULTIFUNCTIONAL ANTIWEAR ADDITIVES**

**BACKGROUND OF THE INVENTION**

**1. Field of the Invention**

This application is directed to alkanol-amine-derived thioesters as multifunctional additives in lubricants and fuels.

**2. Description of Related Art**

Sulfur-containing compounds have been known to provide antiwear properties on metal parts in lubricants. The protection is believed to come from surface-active sulfur groups and other functionalities which may be induced to form a preferable conformation under service conditions U.S. Pat. No. 4,863,534 describes secondary and tertiary alkanol amines as being useful in the preparation of solubilizers useful in dispersing oil-soluble, water-insoluble functional additives in water-based functional fluids.

Now, thioesters derived from alkanol amines have been found to provide superior multifunctional antiwear performance with potential antifatigue, anticorrosion, antirust, cleanliness and thermal stabilizing/antioxidant characteristics.

**BRIEF SUMMARY OF THE INVENTION**

The present invention is directed to amine-derived thioesters as highly efficient multifunctional antiwear additives for various lubricants. More particularly, the additives in accordance with the present invention are derived from dialkanol- and trialkanol amines and a suitable sulfur source. These additives are also believed to be useful in hydrocarbyl or hydrocarboxy fuels.

An object of this invention is to provide improved lubricant and fuel compositions comprising a major amount of said lubricant or fuel and a minor amount of the aforementioned alkanol amine-derived thioester additives.

**DESCRIPTION OF THE PREFERRED  
EMBODIMENTS**

A preferred preparation of the subject amine-derived thioesters is described in FIGS. 1 and 2 below.



-continued



Where n equals 1-100 and preferably 1 or 2.

R equals C<sub>1</sub> to about C<sub>60</sub>, preferably C<sub>12</sub> to about C<sub>18</sub>.

Suitable alkanolamines include but are not limited to the following: triethanol amine, diethanol amine, di-propanol amine, tripropanol amine and the like, bis-(hydroxyethyl)-cocoamine and the like.

Any suitable sulfur source may be used. However, mercaptans or mercapto-derived compounds which contain at least one carboxylic functionality are preferred. Useful sulfur sources include but are not limited to the following: thioglycolic acid, 3-mercaptopropionic acid, thiolactic acid, thiomalic acid, dithiodiglycolic acid, thioglycolic acid, and thiadipropionic acid.

25

Conditions for the above reactions may vary widely depending upon specific reactants, the presence or absence of a solvent and the like. Any suitable set of reaction conditions known to the art may be used. Generally stoichiometric quantities of reactants are used. However, more than molar or less than molar or equimolar amounts may be used. The reaction conditions may vary as follows: the reaction temperature may vary from ambient or 25° C. to about 300° C., the pressure may vary from ambient or about 1 atm to about 10 atm and the molar ratio of reactants preferably varies from about 1:10 moles to about 10:1 moles of alkanol amine to sulfur source.

30

35

40

45

50

55

The additives embodied herein are utilized in lubricating oil or grease compositions in an amount which imparts significant antiwear characteristics to the oil or grease as well as reducing the friction of engines operating with the oil in its crankcase. Concentrations of about 0.001 to about 10 wt. % based on the total weight of the composition can be used. Preferably, the concentration is from 0.1 to about 3 wt. %. It is expected that these materials would also be suitable for use in liquid hydrocarbyl or alcoholic or mixed hydrocarbyl/alcoholic or oxygenated fuel compositions. They are utilized in fuels in amounts of from about 25 to 500 pounds of additive per thousand barrels of fuel and preferably from about 50 to about 250 pounds per 1000 barrels of fuel.

The additives have the ability to improve the above noted characteristics of various oleaginous materials such as hydrocarbyl lubricating media which may comprise liquid oils in the form of either a mineral oil or a synthetic oil, or in the form of a grease in which the aforementioned oils are employed as a vehicle.

60

65

In general, mineral oils, both paraffinic, naphthenic and mixtures thereof, employed as the lubricant, or grease vehicle, may be of any suitable lubricating viscosity range, as for example, from about 45 SSU at 100° F. to about 6000 SSU at 100° F. and preferably, from about 50 to about 250 SSU at 210° F. These oils may have viscosity indexes ranging to about 95 are preferred. The average molecular weights of these oils may range from about 250 to about 800. Where the lubricant is to be employed in the form of a grease, the lubricating oil is generally employed in an amount sufficient to balance the total grease composition, after accounting for the desired quantity of the thickening agent, and

other additive components to be included in the grease formulation.

A wide variety of materials may be employed as thickening or gelling agents. These may include any of the conventional metal salts or soaps, which are dispersed in the lubricating vehicle in grease-forming quantities in an amount to impart to the resulting grease composition the desired consistency. Other thickening agents that may be employed in the grease formulation may comprise the non-soap thickeners, such as surface-modified clays and silicas, aryl ureas, calcium complexes and similar materials. In general, grease thickeners may be employed which do not melt and dissolve when used at the required temperature within a particular environment; however, in all other respects, any materials which is normally employed for thickening or gelling hydrocarbon fluids for foaming grease can be used in preparing grease in accordance with the present invention.

In instances where synthetic oils, or synthetic oils employed as the lubricant or vehicle for the grease, are desired in preference to mineral oils, or in combination therewith, various compounds of this type may be successfully utilized. Typical synthetic oils include, but are not limited to, polyisobutylene, polybutenes, hydrogenated polydecenes, polypropylene glycol, polyethylene glycol, trimethylpropane esters, neopentyl and pentamethylol esters, di(2-ethylhexyl) sebacate, di(2-ethylhexyl) adipate, dibutyl phthalate, fluorocarbons, silicate esters, silanes, esters of phosphorus-containing acids, liquid ureas, ferrocene derivatives, hydrogenated synthetic oils, chain-type polyphenyls, siloxanes and silicones (polysiloxanes), alkyl-substituted diphenyl ethers typified by a butyl-substituted bis(p-phenoxy phenyl) ether, phenoxy phenylethers. Ester-based lubricants are highly suitable.

The fuels contemplated are liquid hydrocarbon combustion fuels, including oxygenated and alcoholic fuels as well as distillate fuels and fuel oils.

It is to be understood, however, that the compositions contemplated herein can also contain other materials. For example, corrosion inhibitors, extreme pressure agents, low temperature properties modifiers and the like can be used as exemplified respectively by metallic phenates sulfonates, polymeric succinimides, non-metallic or metallic phosphorodithioates and the like. These materials do not detract from the value of the compositions of this invention, rather the materials serve to impart their customary properties to the particular compositions in which they are incorporated.

The following examples are merely illustrative and not meant to be limitations.

#### EXAMPLE 1

A solution of bis-(hydroxyethyl)cocoamine (100 g, 0.37 mol) in 100 ml toluene was prepared in a stirred glass reactor equipped with heater, condenser and Dean-Stark trap. Mercaptoacetic acid (67 g, 0.73 mol) was then added to the reactor solution. The solution was refluxed for 4 hours or until 13 ml H<sub>2</sub>O was collected in the Dean-Stark trap. The solvent was evaporated under a reduced pressure to afford the product as a yellowish oil (151 g).

#### EXAMPLE 2

A solution of triethanol amine (100 g, 0.67 mol) in 150 ml toluene was prepared in a stirred glass reactor equipped with heater, condenser and Dean-Stark trap.

Mercaptoacetic acid (185 g, 2.0 mol) was then added to the reactor solution. The solution was refluxed for 5 hours or until 36 ml H<sub>2</sub>O was collected in the Dean-Stark trap. The solvent was evaporated under a reduced pressure to afford the product as a yellowish oil (240 g).

#### EVALUATION

The thioketals thus obtained were blended into mineral oils and evaluated using the Four-Ball Wear Test at 60 kg load/2000 rpm/200° F. for 30 min (Table 1).

In the Four Ball Test three stationary balls are placed in a lubricant cup and a lubricant containing the compound to be tested is added thereto, and a fourth ball is placed in a chuck mounted on a device which can be used to spin the ball at known speeds and loads. The examples were tested using half inch stainless steel balls for thirty minutes under 60 kg load at 2000 rpm and 200° F. If additional information is desired consult test method ASTM D2266 and/or U.S. Pat. No. 4,761,482.

TABLE 1

| Item                                                                                        | Additive Concentration, wt % | Wear Scar Diameter, mm        |      |
|---------------------------------------------------------------------------------------------|------------------------------|-------------------------------|------|
|                                                                                             |                              | 60 kg/2000 rpm/30 min/200° F. | 3.29 |
| Base Oil (80% solvent paraffinic bright, and 20% solvent paraffinic neutral lubricant oils) | —                            |                               |      |
| Example 1 in above oil                                                                      | 1.0                          | 1.46                          |      |
| Example 2 in above oil                                                                      | 1.0                          | 0.80                          |      |

The Four-Ball Wear Test results demonstrate the excellent antiwear properties of these compositions when used at only 1% concentration in mixed mineral oils.

Thioesters derivatized from amines are an entirely new class of compounds which exhibit good antiwear properties in mineral oils under severe service conditions as exemplified by the above test data. These properties enhance the antiwear characteristics of premium quality automotive and industrial lubricants and extend their service life. These compounds can be easily manufactured with known additive technologies and also advance next-generation, premium quality, automotive and industrial lubricants, greases and fuels.

Although the present invention has been described with preferred embodiments, it is to be understood that modifications and variations may be resorted to, without departing from the spirit and scope of this invention, as those skilled in the art will readily understand. Such variations and modifications are considered within the purview and scope of the appended claims.

We claim:

1. An improved lubricant composition comprising a major proportion of said lubricant and a minor proportion of a multifunctional antiwear additive product of reaction prepared from the reaction of a suitable sulfur-containing compound selected from the group consisting of mercaptans and mercapto-derived compounds which contain at least one carboxylic functionality and an alkanol amine in molar ratios varying from 1:10 to 10:1 of alkanol amine to sulfur compound at temperatures varying from ambient to about 300° C. under pressures varying from ambient to 10 atm for a time sufficient to obtain an amine-derived thioester additive product of reaction.
- 60 65 66 67 68 69 70 71 72 73 74 75 76 77 78 79 80 81 82 83 84 85 86 87 88 89 90 91 92 93 94 95 96 97 98 99 100 101 102 103 104 105 106 107 108 109 110 111 112 113 114 115 116 117 118 119 120 121 122 123 124 125 126 127 128 129 130 131 132 133 134 135 136 137 138 139 140 141 142 143 144 145 146 147 148 149 150 151 152 153 154 155 156 157 158 159 160 161 162 163 164 165 166 167 168 169 170 171 172 173 174 175 176 177 178 179 180 181 182 183 184 185 186 187 188 189 190 191 192 193 194 195 196 197 198 199 200 201 202 203 204 205 206 207 208 209 210 211 212 213 214 215 216 217 218 219 220 221 222 223 224 225 226 227 228 229 230 231 232 233 234 235 236 237 238 239 240 241 242 243 244 245 246 247 248 249 250 251 252 253 254 255 256 257 258 259 260 261 262 263 264 265 266 267 268 269 270 271 272 273 274 275 276 277 278 279 280 281 282 283 284 285 286 287 288 289 290 291 292 293 294 295 296 297 298 299 300 301 302 303 304 305 306 307 308 309 310 311 312 313 314 315 316 317 318 319 320 321 322 323 324 325 326 327 328 329 330 331 332 333 334 335 336 337 338 339 340 341 342 343 344 345 346 347 348 349 350 351 352 353 354 355 356 357 358 359 360 361 362 363 364 365 366 367 368 369 370 371 372 373 374 375 376 377 378 379 380 381 382 383 384 385 386 387 388 389 390 391 392 393 394 395 396 397 398 399 400 401 402 403 404 405 406 407 408 409 410 411 412 413 414 415 416 417 418 419 420 421 422 423 424 425 426 427 428 429 430 431 432 433 434 435 436 437 438 439 440 441 442 443 444 445 446 447 448 449 450 451 452 453 454 455 456 457 458 459 460 461 462 463 464 465 466 467 468 469 470 471 472 473 474 475 476 477 478 479 480 481 482 483 484 485 486 487 488 489 490 491 492 493 494 495 496 497 498 499 500 501 502 503 504 505 506 507 508 509 510 511 512 513 514 515 516 517 518 519 520 521 522 523 524 525 526 527 528 529 530 531 532 533 534 535 536 537 538 539 540 541 542 543 544 545 546 547 548 549 550 551 552 553 554 555 556 557 558 559 560 561 562 563 564 565 566 567 568 569 570 571 572 573 574 575 576 577 578 579 580 581 582 583 584 585 586 587 588 589 5810 5811 5812 5813 5814 5815 5816 5817 5818 5819 5820 5821 5822 5823 5824 5825 5826 5827 5828 5829 5830 5831 5832 5833 5834 5835 5836 5837 5838 5839 5840 5841 5842 5843 5844 5845 5846 5847 5848 5849 5850 5851 5852 5853 5854 5855 5856 5857 5858 5859 5860 5861 5862 5863 5864 5865 5866 5867 5868 5869 58610 58611 58612 58613 58614 58615 58616 58617 58618 58619 58620 58621 58622 58623 58624 58625 58626 58627 58628 58629 58630 58631 58632 58633 58634 58635 58636 58637 58638 58639 58640 58641 58642 58643 58644 58645 58646 58647 58648 58649 58650 58651 58652 58653 58654 58655 58656 58657 58658 58659 58660 58661 58662 58663 58664 58665 58666 58667 58668 58669 58670 58671 58672 58673 58674 58675 58676 58677 58678 58679 58680 58681 58682 58683 58684 58685 58686 58687 58688 58689 58690 58691 58692 58693 58694 58695 58696 58697 58698 58699 586100 586101 586102 586103 586104 586105 586106 586107 586108 586109 586110 586111 586112 586113 586114 586115 586116 586117 586118 586119 586120 586121 586122 586123 586124 586125 586126 586127 586128 586129 586130 586131 586132 586133 586134 586135 586136 586137 586138 586139 586140 586141 586142 586143 586144 586145 586146 586147 586148 586149 586150 586151 586152 586153 586154 586155 586156 586157 586158 586159 586160 586161 586162 586163 586164 586165 586166 586167 586168 586169 586170 586171 586172 586173 586174 586175 586176 586177 586178 586179 586180 586181 586182 586183 586184 586185 586186 586187 586188 586189 586190 586191 586192 586193 586194 586195 586196 586197 586198 586199 586200 586201 586202 586203 586204 586205 586206 586207 586208 586209 586210 586211 586212 586213 586214 586215 586216 586217 586218 586219 586220 586221 586222 586223 586224 586225 586226 586227 586228 586229 586230 586231 586232 586233 586234 586235 586236 586237 586238 586239 586240 586241 586242 586243 586244 586245 586246 586247 586248 586249 586250 586251 586252 586253 586254 586255 586256 586257 586258 586259 586260 586261 586262 586263 586264 586265 586266 586267 586268 586269 586270 586271 586272 586273 586274 586275 586276 586277 586278 586279 586280 586281 586282 586283 586284 586285 586286 586287 586288 586289 586290 586291 586292 586293 586294 586295 586296 586297 586298 586299 586300 586301 586302 586303 586304 586305 586306 586307 586308 586309 586310 586311 586312 586313 586314 586315 586316 586317 586318 586319 586320 586321 586322 586323 586324 586325 586326 586327 586328 586329 586330 586331 586332 586333 586334 586335 586336 586337 586338 586339 586340 586341 586342 586343 586344 586345 586346 586347 586348 586349 586350 586351 586352 586353 586354 586355 586356 586357 586358 586359 586360 586361 586362 586363 586364 586365 586366 586367 586368 586369 586370 586371 586372 586373 586374 586375 586376 586377 586378 586379 586380 586381 586382 586383 586384 586385 586386 586387 586388 586389 586390 586391 586392 586393 586394 586395 586396 586397 586398 586399 586400 586401 586402 586403 586404 586405 586406 586407 586408 586409 586410 586411 586412 586413 586414 586415 586416 586417 586418 586419 586420 586421 586422 586423 586424 586425 586426 586427 586428 586429 586430 586431 586432 586433 586434 586435 586436 586437 586438 586439 586440 586441 586442 586443 586444 586445 586446 586447 586448 586449 586450 586451 586452 586453 586454 586455 586456 586457 586458 586459 586460 586461 586462 586463 586464 586465 586466 586467 586468 586469 586470 586471 586472 586473 586474 586475 586476 586477 586478 586479 586480 586481 586482 586483 586484 586485 586486 586487 586488 586489 586490 586491 586492 586493 586494 586495 586496 586497 586498 586499 586500 586501 586502 586503 586504 586505 586506 586507 586508 586509 586510 586511 586512 586513 586514 586515 586516 586517 586518 586519 586520 586521 586522 586523 586524 586525 586526 586527 586528 586529 586530 586531 586532 586533 586534 586535 586536 586537 586538 586539 586540 586541 586542 586543 586544 586545 586546 586547 586548 586549 586550 586551 586552 586553 586554 586555 586556 586557 586558 586559 586560 586561 586562 586563 586564 586565 586566 586567 586568 586569 586570 586571 586572 586573 586574 586575 586576 586577 586578 586579 586580 586581 586582 586583 586584 586585 586586 586587 586588 586589 586590 586591 586592 586593 586594 586595 586596 586597 586598 586599 586600 586601 586602 586603 586604 586605 586606 586607 586608 586609 586610 586611 586612 586613 586614 586615 586616 586617 586618 586619 586620 586621 586622 586623 586624 586625 586626 586627 586628 586629 586630 586631 586632 586633 586634 586635 586636 586637 586638 586639 586640 586641 586642 586643 586644 586645 586646 586647 586648 586649 586650 586651 586652 586653 586654 586655 586656 586657 586658 586659 586660 586661 586662 586663 586664 586665 586666 586667 586668 586669 586670 586671 586672 586673 586674 586675 586676 586677 586678 586679 586680 586681 586682 586683 586684 586685 586686 586687 586688 586689 586690 586691 586692 586693 586694 586695 586696 586697 586698 586699 586700 586701 586702 586703 586704 586705 586706 586707 586708 586709 586710 586711 586712 586713 586714 586715 586716 586717 586718 586719 586720 586721 586722 586723 586724 586725 586726 586727 586728 586729 586730 586731 586732 586733 586734 586735 586736 586737 586738 586739 586740 586741 586742 586743 586744 586745 586746 586747 586748 586749 586750 586751 586752 586753 586754 586755 586756 586757 586758 586759 586760 586761 586762 586763 586764 586765 586766 586767 586768 586769 586770 586771 586772 586773 586774 586775 586776 586777 586778 586779 586780 586781 586782 586783 586784 586785 586786 586787 586788 586789 586790 586791 586792 586793 586794 586795 586796 586797 586798 586799 586800 586801 586802 586803 586804 586805 586806 586807 586808 586809 586810 586811 586812 586813 586814 586815 586816 586817 586818 586819 586820 586821 586822 586823 586824 586825 586826 586827 586828 586829 586830 586831 586832 586833 586834 586835 586836 586837 586838 586839 586840 586841 586842 586843 586844 586845 586846 586847 586848 586849 586850 586851 586852 586853 586854 586855 586856 586857 586858 586859 586860 586861 586862 586863 586864 586865 586866 586867 586868 586869 586870 586871 586872 586873 586874 586875 586876 586877 586878 586879 586880 586881 586882 586883 586884 586885 586886 586887 586888 586889 586890 586891 586892 586893 586894 586895 586896 586897 586898 586899 586900 586901 586902 586903 586904 586905 586906 586907 586908 586909 586910 586911 586912 586913 586914 586915 586916 586917 586918 586919 586920 586921 586922 586923 586924 586925 586926 586927 586928 586929 586930 586931 586932



where  $n = 1-100$

and wherein  $R = C_1$  to about  $C_{60}$ .

3. The composition of claim 1 wherein the product has the following structural formula:



Where  $n = 1-100$ .

4. The composition of claim 1 wherein an amine-derived thioester is prepared from the reaction of bis(hydroxyethyl)cocoamine and mercaptoacetic acid.

5. The composition of claim 1 wherein an amine-derived thioester is prepared from the reaction of triethanol amine and mercaptoacetic acid.

6. The composition of claim 1 wherein the lubricant is an oil of lubricating viscosity selected from the group consisting of (1) mineral oils, (2) synthetic oils, (3) or mixtures of mineral and synthetic oils or is (4) a grease prepared from any one of (1), (2) or (3).

7. The composition of claim 6 wherein the lubricant contains from about 0.001 to about 10 wt % based on 35 the total weight of the composition of the additive product of reaction.

8. The composition of claim 6 wherein the lubricant is a synthetic oil.

9. A process of preparing a multifunctional antioxidant, antiwear additive product prepared by reacting a suitable sulfur-containing compound selected from the group consisting of mercaptans and mercapto-derived compounds which contain at least one carboxylic functionality and an alkanol amine in molar ratios varying from 1:10 to 10 to 1 of alkanol amine to sulfur compound at temperatures varying from ambient to about 300° C. under pressures varying from ambient or 1 atm 45

to about 10 atm for a time sufficient to obtain an amine-derived thioester additive product of reaction.

10. The process of claim 9 wherein the product has the following generalized structure:

5



Where  $n = 1-100$

15 and wherein  $R = C_1$  to about  $C_{60}$ .

11. The process of claim 9 wherein the product has the following generalized structure:

20



Where  $n = 1-100$ .

12. The process of claim 9 wherein an amine-derived thioester is prepared from the reaction of bis(hydroxyethyl)cocoamine and mercaptoacetic acid.

13. The product of reaction prepared in accordance with claim 9 wherein an amine derived thioester is prepared from the reaction of triethanol amine and mercaptoacetic acid.

14. A product of reaction prepared in accordance with claim 9 wherein the product has the following generalized structural formula:

30



40 Where  $n = 1-100$ .

15. A method of preparing an improved lubricant composition comprising adding to said lubricant a minor multifunctional antioxidant and/or antiwear amount of a product of reaction as described in claim 9.

45 16. The method of claim 15 wherein said minor amount is from about 0.001 to about 10 wt % based on the total weight of the composition of said additive product of reaction.

\* \* \* \* \*

50

55

60

65